

1

2,856,315

## FLEXIBLE HARD SURFACE FLOOR AND WALL COVERINGS AND PROCESS THEREFOR

Theodore L. Kuder, Media, and Richard W. Reaves, Chester, Pa., assignors to Congoleum-Nairn Inc., Kearny, N. J., a corporation of New York

No Drawing. Application August 4, 1954  
Serial No. 447,898

19 Claims. (Cl. 117—76)

This invention relates to flexible, hard surface floor and wall covering products of the printed felt base type which are comprised of a backing or base material of impregnated felt on which a wear layer and design has been applied with an oleoresinous and/or alkyd paint.

Any raw felt suitable for use in the production of printed felt base floor coverings can be saturated with any of a number of saturants, including bituminous materials such as asphalt, and synthetic resins such as butadiene-styrene copolymers, chloroprene polymers, and the like. Such saturated felts may be prepared by passing a sheet of raw felt through a tank containing the saturant; or if desired, the saturant may be deposited upon the fibers in a beater in accordance with well-known beater-saturating techniques. The use of beater-saturation is particularly desirable when the saturant is a synthetic resin. After saturation of the felt material, it is simply necessary to permit the saturant to dry prior to conventional use.

In preparing the type of floor and wall covering products with which the present invention is concerned, it has been found necessary to apply one or more coats of a sealing material to the impregnated felt prior to providing a design and wear layer thereon. The seal coat serves a dual purpose of minimizing the tendency of some impregnants to migrate from within and on the felt into the wear layer of the product and to provide a smooth surface on which to deposit the wear layer. Oleoresinous compositions based on drying oils, resins, fillers and/or pigments are most frequently used for this purpose. Elastomeric material such as styrene-butadiene, acrylonitrile-butadiene, isobutylene-isoprene, polychloroprene and the like have been reported to be suitable for use as impregnated felt seal coats where it is desired to deposit thereon a design and wear layer of thermoplastic vinyl materials such as vinyl chloride. The present invention, however, as aforementioned, is concerned only with the problem of depositing a wear layer and design on impregnated felt with an oleoresinous and/or alkyd type paint.

Oleoresinous print paints, like oleoresinous seal coat paints, are comprised of a drying or semi-drying oil base, usually fortified with a resinous material such as rosin, terpene resins, phenol formaldehyde resins, alkyd resins and the like, which function as a binder for pigments and suitable fillers such as titanium dioxide, calcium carbonate, silicates and the like. Drying agents, accelerators, solvents, and the like are usually employed for their specific functions in accordance with the well-known practices in the art. Alkyd print paints are similar to oleoresinous print paints except that an alkydresin is employed in the binder instead of or in conjunction with a drying oil.

Oleoresinous and alkyd paints, hard surface flexible floor and wall covering felts, felt impregnants, oleoresinous, alkyd and elastomeric seal coats are all well known in the arts, many of them having been in use between fifty and a hundred years.

2

In the past, seal coats of the oleoresinous and alkyd type have proved particularly unsatisfactory in regard to decreased distensibility and stiffening during storage with the consequent development of a brittle product. Printed felt base made in the conventional manner exhibits a marked decrease in distensibility in a period as short as one month as compared to its distensibility at the time of production. The problem is aggravated under storage conditions wherein elevated temperatures on the order of 100° F. are experienced. It is believed that this characteristic of printed felt base products which have one or more oleoresinous and/or alkyd seal coats is due to oxidation and/or polymerization of the seal coat compositions which begin at the time of application, continue during storage and are accelerated by elevated temperatures. In connection with narrower widths of printed felt base, decreased distensibility is not a serious problem as the goods are not ordinarily subjected to severe bending and flexing in use. In connection with the wider products, however, the problem becomes acute resulting in cracking and breaking in the course of unrolling or under other conditions normally experienced in handling and installing the goods.

A standard test for measuring the distensibility of printed felt base is reported in U. S. Government Specifications for Felt Backed Flooring LLL-F-471 and Federal Specifications LLL-L-351a, LLL-L-359 and LLL-L-367. The test requires that strips of printed felt base measuring 3 inches by 15 inches be placed over 180° of mandrels of varying diameters. The diameter of the last mandrel upon which the strip is placed immediately prior to cracking on the next succeeding smaller mandrel is reported in inches as the measure of distensibility. Mandrel diameters begin at  $\frac{1}{4}$  inch and increase by increments on the order of  $\frac{1}{2}$  inch until larger diameters of about 2 inches are reached and thereafter the diameters increase at 1 inch intervals. Prior to the test any material to be tested is conditioned for 24 hours at about 23° C. and 50% R. H. Experience has indicated that a mandrel test reading of 1.5 at the time of manufacture is preferred because of an anticipated reasonable storage period of from 9 to 12 months. During this time the printed felt base products of the prior art exhibit a marked decrease in distensibility. If the initial mandrel test reading is 2 or more, the rate of decrease has been found to be greater than the rate of decrease of a product having an initial reading of 1.5 or less.

Another test has been developed to measure the distensibility of printed felt base surface covering which is believed to be a more practical reflection of this characteristic. It is referred to as the "unsupported bend test" and employs an instrument having gripping means spaced 7 inches apart and adapted to concurrently move at a slow speed toward a center point. A strip of printed felt base 9 inches long is placed in the gripping means which are thereafter caused to begin movement. The movement automatically stops at a point where the first cracking occurs on the surface of the printed felt base under test. The distance in inches between the gripping means at that time represents the measure of distensibility of the product.

While the industry has experienced only limited difficulty in providing acceptable products where at least one dimension of the products was less than about 9 feet, it has not been able to continuously stay within acceptable standards of distensibility for wider products. For this reason, many attempts have been made to replace the oleoresinous seal coat with some other material which is capable of functioning as a seal coat, but which provides, in addition, the desired distensibility characteristics at a reasonable cost.

Such attempts have included the use of elastomeric

base seal coats, which, however, proved unacceptable at the outset because of the resultant unsatisfactory appearance of the wear layer deposited thereon. It appears that numerous tiny raised points cover the surface of the oleoresinous or alkyd print paint surface after it has been applied to an elastomeric seal coat surface and dried; however, these apparent raised portions of the paint cannot be felt even with the most sensitive instruments. Some scientists are of the opinion that it is an optical rather than a physical phenomenon. Exaggerated occurrences of this condition bear a resemblance to the rind or peel of an orange; and, in fact, it is referred to in the industry as "orange peel." The reason for the development of "orange peel" is unknown; however, it is usually associated with a combination of elastomeric and oleoresinous and/or alkyd layers of material, and only infrequently appears in connection with the usual type of seal coat and print paint.

It is an object of the present invention to provide a printed felt base product having improved distensibility at the time of production, and one which does not embrittle beyond the point of acceptability in the course of storage. Another object is to provide such a product which exhibits a minimum amount of "orange peel." It is also an object to achieve the above results without effecting any product quality deterioration, and in fact, to achieve certain quality improvements by way of greater distensibility at little or no cost increase. These and other objects will become apparent from the following detailed description of the invention.

It has now been discovered that the above and other objects are achieved by seal coating impregnated felt first with a synthetic elastomeric material, and thereafter with an oleoresinous and/or alkyd material prior to printing with an oleoresinous and/or alkyd paint.

All synthetic elastomeric materials are suitable for use in the present invention. Examples of such materials are: internally or post plasticized copolymers of polyvinyl acetate and acrylic esters, the half butyl esters of maleic anhydride and polyvinyl chloride, copolymers of acrylic acid esters, copolymers of acrylonitrile and butadiene, copolymers of polyvinylidene chloride, the internal or post plasticized homopolymer of polystyrene, the tripolymer of acrylonitrile and butadiene, polyvinyl acetate, and styrene-butadiene. Of these the styrene-butadiene elastomers are preferred because they provide the greatest amount of distensibility in the final product at the time of production and after considerable periods of storage. They make possible the greatest amount of reduction of, or the elimination of, the development of "orange peel." In addition, they provide a superior bond between the impregnated felt and the first seal coat, as well as between the first seal coat and the second seal coat of oleoresinous and/or alkyd material. It has been found that of the styrene-butadienes those having a ratio of from about 65% to about 50% polystyrene to from about 35% to about 50% butadiene are preferred in regard to the final product characteristic aforementioned. A ratio of about 60% polystyrene to about 40% butadiene is most preferred in that nearly complete elimination of "orange peel" is made possible and a greatly improved distensibility is effected. A styrene-butadiene elastomer containing more than 65% polystyrene is less distensible than the preferred product while the same elastomer containing less than 50% polystyrene results in staining of the printed final layer by certain impregnants particularly those of the bituminous type.

The amount of elastomeric material to be used in the first coat composition is critical. If it comprises less than about 10% of the total solids of the seal coat, a discontinuous film or coating will be obtained. If, on the other hand, it exceeds about 25%, the coating will not function as a sealer for the bituminous type impregnants and in addition will increase the cost of the product so as to render it non-competitive. It is preferred that the

binder constitute from about 12% to about 15% of the solids in the composition.

The other ingredients of the elastomer base seal coat composition are those normally found in oleoresinous seal coats. Fillers, such as calcium carbonate, silicates, mica, clay, and the like are employed in conjunction with small amounts of additives such as pigments, anticoagulants, dispersing agents, and the like. Since the surface tension of a composition as described above is relatively high and therefore conducive to the entrapment of small air bubbles and the subsequent creation of "craters" and "pin holes" in the final print paint layer, it is preferred that a surface tension reducing agent be employed. A small amount of a material such as a limed rosin-linseed oil varnish, casein, or lecithin has been found to be excellent for this purpose; however, any drying oil or resin may be used. The surface tension reducing agent generally serves as a binder in addition to the elastomeric material, and therefore, reference herein to the first coat binder is meant to include both the elastomeric material and any surface tension reducing agent which also functions as a binder. Generally, the ratio of elastomeric material to surface tension reducing material should be between about 18 to 1 and about 3 to 1 depending on the surface tension reducing agent selected. In the case of linseed oil—rosin varnish 9 to 1 is the preferred ratio. Since the above mentioned additives constitute only a minor portion of the elastomer base first coat composition, all reference to fillers in the present specification and the claims is meant to include such additives unless otherwise indicated.

In preparing a composition as described above, it is preferred to first prepare an emulsion of the elastomeric material. The manner of accomplishing this is well known and is fully described in U. S. Patent No. 2,498,712 to Ryden and U. S. Patent No. 2,386,764 to Zwicker. Such emulsions usually contain emulsifying agents, i. e., casein, lecithin, and the like, as well as from about 40% to about 60% water. All of the ingredients set forth above may simply be well mixed with the emulsion of elastomeric material while making provision for maintaining a pH in the entire mixture between about 8.5 and 9.5, thereby preventing coagulation of the elastomer. The pH adjustment usually must be directed upwardly and therefore a basic material such as ammonium hydroxide may be employed for this purpose.

The following examples are typical compositions which may be employed as the first seal coat of the invention. The total amount of water is governed only by the means which are selected to apply the seal coat to the impregnated felt base.

#### EXAMPLE 1

|                                                                     | Parts |
|---------------------------------------------------------------------|-------|
| Calcium carbonate                                                   | 695   |
| Iron oxide (pigment)                                                | 5     |
| Tetra sodium pyrophosphate (anticoagulant and dispersing agent)     | 4     |
| Butadiene-styrene latex (48% solids; 40% butadiene-60% polystyrene) | 180   |
| Rosin-linseed oil varnish                                           | 10    |
| Ammonium hydroxide                                                  | 2     |
| Water                                                               | 110   |

#### EXAMPLE 2

|                                     |     |
|-------------------------------------|-----|
| Mica-clay-calcium carbonate mixture | 670 |
| Polyvinyl acetate (50% solids)      | 240 |
| Casein                              | 10  |
| Ammonium hydroxide                  | 1   |
| Water                               | 110 |

#### EXAMPLE 3

|                                                   |     |
|---------------------------------------------------|-----|
| Calcium carbonate                                 | 640 |
| Copolymer of polyvinylidene chloride (50% solids) | 300 |
| Soya lecithin                                     | 10  |
| Ammonium hydroxide                                | 1   |
| Water                                             | 110 |

## 5

## EXAMPLE 4

|                                                                | Parts |
|----------------------------------------------------------------|-------|
| Calcium carbonate                                              | 670   |
| Internally plasticized homopolymer of polystyrene (40% solids) | 300   |
| Rosin-linseed oil varnish                                      | 10    |
| Ammonium hydroxide                                             | 1     |
| Water                                                          | 110   |

## EXAMPLE 5

|                                                                                      |     |
|--------------------------------------------------------------------------------------|-----|
| Mica-clay-calcium carbonate                                                          | 670 |
| Internally plasticized copolymer of polyvinyl acetate and acrylic ester (50% solids) | 240 |
| Rosin-linseed oil varnish                                                            | 10  |
| Ammonium hydroxide                                                                   | 2   |
| Water                                                                                | 110 |

## EXAMPLE 6

|                                                                          |     |
|--------------------------------------------------------------------------|-----|
| Calcium carbonate                                                        | 640 |
| Half butyl ester of maleic anhydride and polyvinyl chloride (50% solids) | 300 |
| Lecithin                                                                 | 10  |
| Ammonium hydroxide                                                       | 1   |
| Water                                                                    | 110 |

## EXAMPLE 7

|                                                       |     |
|-------------------------------------------------------|-----|
| Clay                                                  | 695 |
| Copolymer of acrylonitrile and butadiene (40% solids) | 250 |
| Iron oxide (pigment)                                  | 5   |
| Ammonium hydroxide                                    | 1   |
| Water                                                 | 110 |

## EXAMPLE 8

|                                                                     |     |
|---------------------------------------------------------------------|-----|
| Calcium carbonate                                                   | 695 |
| Butadiene-styrene latex (50% solids; 50% butadiene-50% polystyrene) | 200 |
| Ammonium hydroxide                                                  | 1   |
| Tetra sodium pyrophosphate (anticoagulant and dispersing agent)     | 4   |
| Water                                                               | 110 |

Example 1 above incorporates the preferred ingredients of the invention in the preferred manner.

The elastomeric seal coat may be applied to the impregnated felt in any suitable manner. Ordinarily it is most easily applied in the form of the above described water emulsions by doctor coating, roller coating or simply by brushing. It has been found, however, that the elastomeric seal coat must be deposited so as to provide a first coat thickness of at least about 4 mils on standard thickness floor covering felt which measures about 0.054 inch. If less than this is applied, the final product will be subject to staining due to the seeping of certain impregnants particularly of the bituminous type. Further, it has been found that if the elastomeric seal coat is applied in an amount less than 4 mils, a discontinuous or spotted final covering results in the final product. It is difficult, moreover, to provide a product having a uniform appearance in regard to gloss if the elastomer seal coat is less than 4 mils in thickness.

In some cases it may be desired to employ a felt base which is thinner or thicker than the aforementioned standard felt measuring 0.054 inch prior to impregnation. Although a linear relationship does not appear to exist between the thickness of the felt and the amount of first seal coat to be applied, it has been found that about 3 mils first coat thickness is satisfactory on a felt measuring 0.020 inch and about 5 mils is satisfactory on a felt measuring 0.060 inch. Part of the function of the first seal coat is to smooth the felt surface and this is not required to as great an extent on thinner felts as it is on thicker felts. It is for this reason that less seal coat is required on the thinner felt material.

The maximum thickness of elastomeric seal coat which may be applied is also critical. If a thickness of 8 mils

## 6

is exceeded, the seal coat develops cracks and fissures. The reason for this is unknown; however, it probably is the result of the bulk of the film at this level. The upper limit remains constant for all thicknesses of felt. The upper limit of first seal coat thickness is of little practical importance because of the cost of material involved.

As aforementioned, it is impossible to print with oleoresinous or alkyd paint directly on an elastomeric material seal coated, impregnated felt without the occurrence of "orange peel," although a considerable amount of improvement in distensibility is effected. In accordance with the present invention, it has been found that a second seal coat of oleoresinous and/or alkyd material greatly minimizes, and in some cases eliminates, the undesirable "orange peel" appearance in the final product while maintaining the principal portion of the increased distensibility which is apparently due to the elastomeric seal coat. The reason for this is unknown since it would be expected that the oleoresinous second coat would result in the same amount of loss of distensibility or embrittling as it did when used in accordance with prior practice.

The second seal coat of oleoresinous material contains the ingredients normally found in oleoresinous seal coats.

As aforementioned, they contain drying oils such as linseed oil, tall oil-linseed oil, soy bean oil-china wood oil, fish oil and the like, and resins such as rosin, ester gum, cumar and the like. Alkyd second coats are similar to oleoresinous second coats except that instead of the oleoresinous materials mentioned above, alkyds are employed. These materials are prepared by cooking the alkyds or drying oil and resin mixtures together, diluting them with solvents and emulsifying them so as to obtain a water in oil paint.

The amount of oleoresinous and/or alkyd second coat to be applied depends to some extent on the amount of binder in the composition. It has been found that the binder must comprise at least about 18% of the coating material in order to obtain a film which is not porous, while it may contain up to about 27% binder without developing an undesirable amount of embrittling during storage of the type which the present invention is directed to overcome. In practice, however, no more than about 25% may be used because of economic considerations.

Within a range of from about 20% to about 24% binder, "orange peel" is greatly minimized, and at the higher levels is substantially completely eliminated, and for these reasons this range is preferred. A composition of the preferred binder content, containing in addition, of course, suitable fillers, may be applied in any manner, such as by doctor coating or by roller coating and the like, and must be applied so as to provide a thickness of about 2 mils. Although it is generally undesirable to decrease this level of second coat because it also has a smoothing function, the binder content may be increased to the higher permissible levels and thereby permit a slight decrease in the second coat thickness. In view of equipment limitations and ease of control, it is preferable to employ a level of about 2 mils. There is no reason to exceed this level as no advantages are obtained thereby.

In preparing the product of the present invention, it is simply necessary to coat the impregnated felt with the first seal coat of elastomeric material and allow it to dry. Thereafter the second seal coat of oleoresinous and/or alkyd material is applied and allowed to dry. The wear layer and design may then be printed on the seal coated felt by conventional printing techniques.

To illustrate the improved characteristics of the products of the present invention, the following mandrel test and unsupported bend tests were conducted. In all cases a control was employed comprising asphalt impregnated felt on which was deposited first a 4 mil layer of a composition consisting of 15% linseed oil-rosin varnish, 82% calcium carbonate and 3% of iron oxide, ammonium hydroxide and soap; second, a 2 mil layer of a com-

position consisting of 21% linseed oil-resin varnish and 79% calcium carbonate; and third, a wear layer and design of oleoresinous print paint. Such controls indicated an average mandrel reading of 1.42 at the time the printed felt base was prepared. The mandrel test reading increased to 2.25 under accelerated storage conditions of one month at 120° F. At the end of six months of actual storage conditions as experienced in the normal channels of commerce, the mandrel test reading averaged 2.0. Table 1 sets forth the comparative mandrel test readings for the 8 elastomeric seal coat examples set forth previously. Table 2 sets forth the unsupported bend test readings for the same products after nine months storage at room temperature. The unsupported bend test reading of the control under the same conditions was 4.5. All of the samples which were tested were comprised of an asphalt impregnated felt backing on which was deposited a 4 mil layer of elastomeric seal coat and a 2 mil layer of 21% binder oleoresinous second coat on which was printed a design with oleoresinous print paint.

Table 1

| Example | At Time of Production | After 1 month at 120° F. | After 6 months Storage | "Orange Peel" |
|---------|-----------------------|--------------------------|------------------------|---------------|
| 1.      | 0.96                  | 1.63                     | 1.50                   | None.         |
| 2.      | 1.0                   | 1.70                     | 1.55                   | Very Slight.  |
| 3.      | 1.1                   | 1.73                     | 1.57                   | Do.           |
| 4.      | 1.0                   | 1.80                     | 1.60                   | None.         |
| 5.      | 1.0                   | 1.75                     | 1.60                   | Very Slight.  |
| 6.      | 1.2                   | 1.80                     | 1.65                   | Slight.       |
| 7.      | 1.0                   | 1.70                     | 1.55                   | None.         |
| 8.      | 1.0                   | 1.70                     | 1.55                   | Do.           |

<sup>1</sup> All readings based on average of 20 samples.

Table 2

| Example | After 9 months Storage | "Orange Peel" |
|---------|------------------------|---------------|
| 1.      | 1.25                   | None.         |
| 2.      | 1.80                   | Very Slight.  |
| 3.      | 1.75                   | Do.           |
| 4.      | 1.50                   | None.         |
| 5.      | 1.60                   | Very Slight.  |
| 6.      | 1.70                   | Slight.       |
| 7.      | 1.40                   | None.         |
| 8.      | 1.40                   | Do.           |

<sup>1</sup> All readings based on average of 20 samples.

While the invention has been described with reference to detailed examples, it is not to be limited thereby. Various changes in formulation and technique may be applied which are within the skill of the art. Reference should be had to the appended claims for the limits of the scope of the invention.

What is claimed is:

1. In a printed felt base surface covering comprising an impregnated felt backing, an oleoresinous seal coat and a decorative wear surface, the improvement which comprises interposing between said felt backing and said oleoresinous seal coat a uniform layer comprising about 10 percent to about 25 percent of a rubbery synthetic elastomer and about 75 percent to about 90 percent filler.
2. In a printed felt base surface covering comprising an impregnated felt backing, an oleoresinous seal coat and a wear surface comprising a dried oleoresinous print paint, the improvement which comprises interposing between said felt backing and said oleoresinous seal coat a uniform layer comprising about 75 percent to about 90 percent filler and about 10 percent to about 25 percent of a butadiene-styrene rubbery elastomer having a ratio of about 1 to about 1.86 parts of polystyrene to 1 part butadiene.
3. In a printed felt base surface covering comprising an impregnated felt backing, an oleoresinous seal coat and a wear surface comprising a dried oleoresinous print paint, the improvement which comprises interposing

between said felt backing and said oleoresinous seal coat a uniform layer comprising about 75 percent to about 90 percent filler and about 10 percent to about 25 percent of a butadiene-styrene rubbery elastomer having a ratio of about 1.5 parts polystyrene to 1 part butadiene.

4. In a printed felt base surface covering comprising an impregnated felt backing, an oleoresinous seal coat and a wear surface comprising a dried oleoresinous print paint, the improvement which comprises interposing between said felt backing and said oleoresinous seal coat a uniform layer comprising about 10 percent to about 25 percent of a butadiene-styrene rubbery elastomer having a ratio of about 1 to about 1.86 parts of polystyrene to 1 part butadiene and about 75 percent to about 90 percent filler, said uniform layer having a thickness in accordance with the following table:

| Thickness of Impregnated Felt | Minimum First Coat Thickness, mils | Maximum First Coat Thickness, mils |
|-------------------------------|------------------------------------|------------------------------------|
| 0.020 inches                  | 3                                  | 8                                  |
| 0.054 inches                  | 4                                  | 8                                  |
| 0.060 inches                  | 5                                  | 8                                  |

5. In a printed felt base surface covering comprising an impregnated felt backing, an oleoresinous seal coat containing about 18 percent to about 27 percent binder and a wear surface comprising a dried oleoresinous print paint, the improvement which comprises interposing between said felt backing and said oleoresinous seal coat a uniform layer comprising about 10 percent to about 25 percent of a rubbery synthetic elastomer selected from the group consisting of plasticized copolymers of polyvinyl acetate and acrylic esters, half butyl esters of maleic anhydride and polyvinyl chloride, copolymers of acrylic acid esters, copolymers of acrylonitrile and butadiene, copolymers of polyvinylidene chloride, plasticized homopolymers of polystyrene, tripolymers of acrylonitrile and butadiene, polyvinyl acetate, and styrene-butadiene and about 75 percent to about 90 percent filler.

6. In a printed felt base surface covering comprising an impregnated felt backing, an oleoresinous seal coat containing 20 percent to 24 percent binder and a wear surface comprising a dried oleoresinous print paint, the improvement which comprises interposing between said felt backing and said oleoresinous seal coat a uniform layer comprising 12 percent to 15 percent butadiene-styrene rubbery elastomer having a ratio of about 1 to about 1.86 parts polystyrene to 1 part butadiene and 85 percent to 88 percent filler.

7. In a printed felt base surface covering comprising an impregnated felt backing, an oleoresinous seal coat and a wear surface comprising a dried oleoresinous print paint, the improvement which comprises interposing between said felt backing and said oleoresinous seal coat a uniform layer comprising about 10 percent to about 25 percent of a mixture of rubbery synthetic elastomer and a compatible surface tension reducing agent and about 75 percent to about 90 percent filler, the ratio of said elastomer to said surface tension reducing agent being about 3 to 1 to about 18 to 1.

8. In a printed felt base surface covering comprising an impregnated felt backing, an oleoresinous seal coat and a wear surface comprising a dried oleoresinous print paint, the improvement which comprises interposing between said felt backing and said oleoresinous seal coat a uniform layer comprising about 10 percent to about 25 percent of a mixture of rubbery synthetic elastomer and a compatible drying oil varnish and about 75 percent to about 90 percent filler, the ratio of said elastomer to said drying oil varnish being about 3 to 1 to about 18 to 1.

9. In a printed felt base surface covering comprising an impregnated felt backing, an oleoresinous seal coat containing about 18 percent to about 27 percent binder and about 73 percent to about 82 percent filler and a

wear surface comprising a dried oleoresinous print paint, the improvement which comprises interposing between said felt backing and said oleoresinous seal coat a uniform layer comprising about 10 percent to about 25 percent of a rubbery synthetic elastomer and about 75 percent to about 90 percent filler.

10. In a seal coated felt for use as a backing for smooth surface coverings comprising impregnated felt and an oleoresinous seal coat, the improvement which comprises interposing between said felt backing and said oleoresinous seal coat a uniform layer comprising about 10 percent to about 25 percent of a rubbery synthetic elastomer and about 75 percent to about 90 percent filler.

11. In a seal coated felt for use as a backing for smooth surface coverings comprising impregnated felt and an oleoresinous seal coat, the improvement which comprises interposing between said felt backing and said oleoresinous seal coat a uniform layer comprising about 10 percent to about 25 percent of a butadiene-styrene rubbery elastomer having a ratio of about 1 to about 1.86 parts of polystyrene to 1 part butadiene and about 75 percent to about 90 percent filler.

12. In a seal coated felt for use as a backing for smooth surface coverings comprising impregnated felt and an oleoresinous seal coat, the improvement which comprises interposing between said felt backing and said oleoresinous seal coat a uniform layer comprising about 10 percent to about 25 percent of a butadiene-styrene rubbery elastomer having a ratio of about 1 to about 1.86 parts of polystyrene to 1 part butadiene and about 75 percent to about 90 percent filler, said uniform layer having a thickness in accordance with the following table:

| Thickness of Impregnated Felt | Minimum First Coat Thickness, mils | Maximum First Coat Thickness, mils |
|-------------------------------|------------------------------------|------------------------------------|
| 0.020 inches.....             | 3                                  | 8                                  |
| 0.034 inches.....             | 4                                  | 8                                  |
| 0.060 inches.....             | 5                                  | 8                                  |

13. In a seal coated felt for use as a backing for smooth surface coverings comprising impregnated felt and an oleoresinous seal coat containing about 18 percent to about 27 percent binder and about 73 percent to about 82 percent filler, the improvement which comprises interposing between said felt backing and said oleoresinous seal coat a uniform layer comprising 12 percent to 15 percent butadiene-styrene rubbery elastomer having a ratio of about 1 to about 1.86 parts polystyrene to 1 part butadiene and 85 percent to 88 percent filler.

14. In a seal coated felt for use as a backing for smooth surface coverings comprising impregnated felt and an oleoresinous seal coat containing about 18 percent to about 27 percent binder and about 73 percent to about 82 percent filler, the improvement which comprises interposing between said felt backing and said oleoresinous

5 seal coat a uniform layer comprising about 10 percent to about 25 percent of a mixture of rubbery synthetic elastomer and a compatible surface tension reducing agent and about 75 percent to about 90 percent filler, the ratio of said elastomer to said surface tension reducing agent being about 3 to 1 to about 18 to 1.

15. In a method of producing a printed felt base surface covering comprising an impregnated felt backing, an oleoresinous seal coat and a wear surface, the improvement which comprises depositing on said felt backing prior to the application of said oleoresinous seal coat a uniform layer comprising about 10 percent to about 25 percent of a rubbery synthetic elastomer and about 75 percent to about 90 percent filler.

16. The method of claim 15 wherein said rubbery synthetic elastomer is a butadiene-styrene rubbery elastomer having a ratio of about 1 to about 1.86 parts polystyrene to about 1 part butadiene.

17. In a method of producing a printed felt base surface covering comprising an impregnated felt backing, an oleoresinous seal coat and a wear surface comprising a dried oleoresinous print paint, the improvement which comprises depositing on said felt backing prior to the application of said oleoresinous seal coat a uniform layer comprising about 10 percent to about 25 percent of a rubbery synthetic elastomer selected from the group consisting of plasticized copolymers of polyvinyl acetate and acrylic esters, half butyl esters of maleic anhydride and polyvinyl chloride, copolymers of acrylic acid esters, 20 copolymers of acrylonitrile and butadiene, copolymers of polyvinylidene chloride, plasticized homopolymers of polystyrene, tripolymers of acrylonitrile and butadiene, polyvinyl acetate, and styrene-butadiene, and about 75 percent to about 90 percent filler.

18. In a method of producing a printed felt base surface covering which comprises an impregnated felt backing, an oleoresinous seal coat containing about 18 percent to about 27 percent binder and a wear surface comprising a dried oleoresinous print paint, the improvement which comprises depositing on said felt backing prior to the application of said oleoresinous seal coat a uniform layer comprising about 10 percent to about 25 percent of a mixture of rubbery synthetic elastomer and a compatible surface tension reducing agent and about 75 percent to about 90 percent filler, the ratio of said elastomer to said surface tension reducing agent being from about 3 to 1 to about 18 to 1.

19. The method according to claim 18 wherein said surface tension reducing agent is a drying oil varnish.

#### References Cited in the file of this patent

#### UNITED STATES PATENTS

|           |                       |               |
|-----------|-----------------------|---------------|
| 2,133,886 | Beegle et al. ....    | Oct. 18, 1938 |
| 2,624,682 | Hazeltine ....        | Jan. 6, 1953  |
| 2,624,683 | Bezman ....           | Jan. 6, 1953  |
| 2,705,683 | Hazeltine et al. .... | Apr. 5, 1955  |
| 2,707,157 | Stanton et al. ....   | Apr. 26, 1955 |